

## UNITED STATES PATENT OFFICE

2,061,211

METHOD OF IMPROVING THE APPEARANCE  
OF SILK FABRICSWarren T. Reddish, Cincinnati, Ohio, assignor  
to Emery Industries, Inc., Cincinnati, Ohio, a  
corporation of OhioNo Drawing. Application January 31, 1933,  
Serial No. 654,554

6 Claims. (Cl. 87—5)

This invention relates to a new art, method, and process of cleaning garments, fabrics, textiles, cloth, rugs and articles of like nature which, for the sake of convenience, throughout the remainder of the description, will be designated by the term "fabrics" unless otherwise specifically identified.

This application is a continuation in part of co-pending application Serial No. 590,981, filed February 4, 1932, and now issued into Patent No. 1,911,289.

In view of the fact that the invention lends itself to being practiced in so-called dry cleaning establishments, on the classes of articles usually cleaned there and with the types of equipment usually used there, the present invention is described and claimed as an improvement in the "dry cleaning" art. However, the physical chemistry utilized in practicing this invention and the results obtained, are so contrary to the principles and go so far beyond results now designated by the term "dry cleaning", that one might classify the fabric cleaning development of this invention as an entirely new art.

In order to comprehend the true novelty of principle of this invention, a brief review of the theories of previously known methods of cleaning fabrics is requisite. Cleaning fabrics has been accomplished in the past either by a soap and water process or by the dry cleaning process. The dry cleaning process differs in principle from the wet washing process.

In the wet washing process the dirt particles on the fabric are removed by emulsification and saponification of the oils and greases which bind the particles to the fabric. This is usually accomplished by washing the fabrics with the ordinary fatty acid soaps which possess emulsifying powers in water solution and liberate alkali by hydrolysis which combines with the saponifiable oils present. These fatty acid soaps also lower the surface tension of the solution which accelerates the detergent action by increasing the rate of penetration of the soap and water into the fabric. The highly water soluble soil which may also be present is removed, of course, by the solvent action of the water. This process is injurious to a majority of types of fabric because it often causes shrinkage, fading or disfigurement.

In the dry cleaning industry to which this invention is directed a conventional cleaning solvent is employed of the type exemplified by a volatile hydrocarbon or chlorinated hydrocarbon, the more commonly used of which are gasoline, naphtha, carbon tetrachloride and trichlor-

ethylene. The term "dry cleaning solvent" will be hereinafter used to designate the class of solvents set forth above. At present, the dry cleaning process is usually practiced by treating the fabrics in rotating drum type washers containing the cleaning solvent to which may be added suitable so-called dry cleaning soaps which decrease static and lower surface tension. The agitation is continued for from ten to thirty minutes, depending upon the type of fabrics being treated and their condition. During this treatment, the oily or greasy film, which binds the dirt particles to the fabrics, is dissolved and the dirt particles are removed by the agitation of the fabrics in the solvent. The articles are then rinsed in clean solvent and centrifugally extracted and then dried either in rotary drum type dryers or in heated rooms. By this treatment oily and greasy soil is removed without shrinkage of the fabric or damage to the sizing and finishing materials, the dyes or the fibre itself.

However, marks or disfigurements called "water spots" which are caused by water having come in contact with the fabric and roughened or partially dissolved the finishing material and spots caused by solely water soluble substances, such as perspiration, soft drinks, sugar syrups, and the like, are not removed by this process. It is, therefore, necessary to employ water or other suitable solvents to remove them. This is usually done by hand spotting of the affected local areas in order that the amount of water coming in contact with the fabric may be kept down to a minimum. Due to the labor involved, this operation is relatively expensive compared to the rest of the process. Moreover, the results obtained depend upon the skill of the worker and, at best, are highly unsatisfactory.

Such spots may in some cases be removed by what is called the wet-dry treatment in which the fabric is first immersed in the cleaning solvent and then, while still saturated with solvent, treated with cold water or a dilute soap solution for from three to five minutes. The presence of the cleaning solvent in the fabric prevents the absorption of sufficient water to cause appreciable shrinking, loss of sizing material or bleeding of colors, but allows the water to come in contact with the soluble spots sufficiently to bring about their solution. This process is tedious, expensive, and may injure a fabric or fail to remove the spots, or both. Obviously, both hand spotting and the wet-dry methods are make-shifts dependent upon artizan skill and judgment. It is, therefore, to be observed at this point that there

is no existing process for cleaning fabrics which is inherently adapted to be used on all types of fabrics to remove all types of soil.

It has always been customary (and still is), 5 to clean fabrics made from vegetable fibres such as cotton and linen goods, by washing in soap and water. This process can also be used on some articles of wool, silk, and rayon, but very great care is required, and generally speaking, the fabrics made from fibre of animal or synthetic origin, 10 which are adapted to the soap and water washing process, are the exception rather than the rule.

Most of the outer garments worn in this country at present, such as suits, dresses, coats, etc., are 15 made from fibres of animal origin, usually silk or wool, or both. Such articles are ruined in appearance by soap and water washing. As a result of the development of cheap cleaning solvents in the last half of the last century, and as a 20 result of the shifting of population to the large urban centers in which more formal attire prevails, the central dry cleaning plant came into being and its facilities became widely available.

The ubiquity of the dry cleaning plants permitted 25 the designers of fabrics to develop a great many new sizing and finishing materials, special weaves, peculiar thread twists, and many new and brilliant dyestuffs, which in cleaning would require the special skill and equipment of the large 30 central dry cleaning establishments. On this account, the so-called dry cleaning process has become a tremendous national industry despite the fact that it does not remove water marks and is inherently adapted to remove from the fabrics 35 but one class of soil, that is, the oil soluble soil, as distinguished from perspiration and other types of water soluble soil.

The object of this invention is to provide an 40 entirely new and novel art, method or process by means of which fabrics are cleansed of substantially all varieties of spots or soil without individual attention to each article treated or the utilization of artizan skill and judgment.

This invention resides in a series of recognitions, 45 concepts and determinations which have required and received verification by large scale commercial operation upon all classes of fabrics normally tendered to dry cleaning establishments throughout the different seasons of the year during 50 which temperature, humidity, the type of garments worn, and the fabrics employed vary substantially.

These recognitions, concepts and determinations are as follows: An optimum cleaning action 55 on fabrics is provided by a cleaning solvent containing a substantial, predetermined and controlled quantity of absorbed moisture. If the moisture be dispersed throughout the cleaning solvent to a very extreme degree, for instance, 60 that degree which is signified by a substantial optical clarity of the solution, then the moisture will not have its usual deleterious effects upon the fibre, the dyestuff, or the finish of the fabric being treated. In other words, even the finest silk 65 evening dress will not be injured by this treatment.

Thus, it is possible to remove the water soluble spots or soil with a quantity of dispersed moisture which is not injurious to the fabric being 70 treated, or vice versa, a quantity of finely dispersed moisture, so small that it does not injure the fabric being treated, has the capacity to remove the water soluble spots and soil. Still otherwise expressed, the invention resides in the concept 75 and determination that an appropriate

amount of moisture appropriately dispersed throughout a dry cleaning solvent, possesses the desirable cleaning properties of water but not the disadvantages.

The next feature of this invention, which is 5 rather unexpected, is that the quantity of moisture adapted to produce the best results should be calculated and controlled primarily in relation to the weight of the fabrics treated, rather than in relation to the weight or quantity of the cleaning 10 solvent used. This is due to the fact that the fabrics always absorb substantially all of the moisture in the cleaning solvent. Therefore, the quantity of moisture contacted with the fabrics or transferred to the fabrics in the process, is the 15 critical factor rather than the ratio of moisture to cleaning solvent in the bath in which the fabrics are treated.

The ratio of moisture to fabric to be used in practicing this invention must depend upon the 20 moisture tolerance of the type of fabric being cleaned. The more specific aspects of the invention may be said to reside in the determination that a useful cleaning action is obtained by agitating the fabrics in a body of cleaning solvent 25 containing about five percent of their weight of moisture and that in many cases, the weight of moisture may be increased to thirty percent of the weight of the fabrics without injury thereto. For instance, silk garments may be cleaned by 30 treatment with between five and fifteen percent of their weight of moisture, though approximately ten percent is recommended for most large scale commercial runs which include numerous evening gowns. In the case of men's suits, ten to 35 thirty percent of their weight of moisture may be used in the cleaning solvent, though fifteen percent seems to produce the best average results on a batch of winter suits collected from a high class suburban neighborhood.

It is obvious that if a fine satin evening dress were treated in a bath in which water and naphtha were simply churned up together, the dress would become hopelessly water spotted because of large drops of water absolutely saturating the 45 dress in many local areas. Such an undesirable effect diminishes in proportion to the fineness of the particles of water. Even a coarse emulsion would ruin a silk dress because the emulsion would saturate completely certain local areas 50 with water and other local areas with the naphtha. If, however, the dispersion of the moisture in the naphtha is so fine that the solution is substantially optically clear, then the absorption of 55 moisture by the fabric being treated is more analogous to the absorption of moisture by a fabric in a very damp climate, for instance, on the seashore.

This new process in which a fabric is treated with and takes on between five and thirty percent of its weight of moisture under normal conditions (a large group of fabrics being churned about in a container of cleaning solvent and moisture), results in the removal from the fabrics of water soluble soil such as syrup spots, perspiration marks, soft drink spots, and the like, as well as all oily or greasy soil. Moreover, water spots disappear from the fabric and many types of finish, in general use at present, seem to be not only completely restored and renovated, but 70 improved by this treatment, so that the fabrics look as well or even better than they did when new.

In view of the fact that moisture does not admix readily with the cleaning solvents in com- 75

mon use at present, absorbefacients must be used—(these will be described at a later point). While the moisture for the first batch of fabrics may be added to the cleaning solvent directly with the absorbefacient, it is believed to be better practice and more in conformity with the spirit of this invention first to add the absorbefacient to the cleaning solvent and thereby create in this cleaning solvent the capacity to absorb the substantial and requisite quantities of moisture in a state sufficiently fine and dispersed as not to be injurious to the fabrics to be treated. Then the desired quantity of moisture may be determined and added for each batch of fabrics treated. This step is termed "humidifying" the cleaning solvent.

It is recommended that the cleaning solvents be constituted water absorbent for the maximum amount of moisture requisite for the impending operations. If this be done, then it is not necessary to adjust the ratio of absorbefacient to cleaning solvent for particular or unusual conditions which may arise.

In commercial operations, each batch of fabrics to be cleaned is weighed. Generally speaking, fifty or sixty pounds of fabric are considered the maximum load for about fifty gallons of cleaning solvent. Then moisture is added to the cleaning solvent, the amount being based upon the weight of fabrics being treated. In this connection, attention should be paid to the humidity of the atmosphere which normally determines the percentage of moisture already in the fabrics. Likewise, it is necessary to take into account the nature of the fabrics being cleaned and the degree of soil.

It is obvious, of course, that fabrics affected by a large amount of exclusively water soluble spots or soil, require treatment with larger quantities of moisture to effect removal than do fabrics having a small amount of soil of this type. When men's rough clothes or the like are being treated, it is possible, if desired, to incorporate so much moisture either before the treatment or during the treatment, that the cleaning solvent becomes murky without injuring the fabrics, though in the case of ladies' fine silk dresses and articles of like nature, injury is almost sure to occur if the dispersion of moisture be coarse. It must be remembered, in this regard, that the optical properties of the solution are mentioned solely for the purpose of indicating the degree of subdivision or dispersion of its moisture content, and that these optical properties have no merit or virtue in and of themselves.

In many climates and cases it is desirable to dry out the fabrics before they are treated, as this step permits the transfer of a larger quantity of moisture to the fabric and hence provides a greater cleaning effect for a given final moisture content of the fabric in question. For instance, if silk garments are being treated and the final moisture content is substantially over fifteen percent, then difficulty is often experienced in the pressing room because of wrinkling. Such garments, however, can be entirely satisfactorily cleaned and pressed first by drying them out, then treating them with about ten percent (based on the weight of the fabrics) of moisture incorporated in the cleaning solvent.

Throughout the claims the terminology "fabric indicated amount of moisture" is used to denote first of all the novel concept of this invention that the amount of moisture employed should be related to the weight of the fabric being

cleaned, the nature of the fabric being cleaned, and the condition of the fabric being cleaned, as distinguished from bearing a predetermined percentage relationship to the cleaning solution as a whole. The selected terminology likewise is employed in the claims to denote the general moisture fabric relationship recommended in the foregoing discussion for operations of the general type specified.

The preferred process, as a series of steps, comprises: First, drying out the fabric to be cleaned, if necessary. Next, the fabrics are weighed. Next, they are given a preliminary dip in a straight solution of cleaning solvent to get off the worst of the dirt and saturate the fibres with cleaning solvent. Next, moisture is introduced into a second batch of cleaning solvent to be used for the crucial treatment, the amount of moisture used being approximately equal to between five and thirty percent of the weight of the fabrics being treated. Ten percent is recommended for fine silks and fifteen percent for men's suits.

After this the fabrics are agitated and churned about in this cleaning bath for a period of between fifteen minutes and half an hour, depending upon the fabrics and their condition. It is highly desirable to filter the cleaning solvent during this cleaning process, in order to prevent dirt particles being loosely deposited upon the fabrics as they are removed from the bath. In view of the fact that most of the filters in use for this purpose do not permit moisture to pass through them, it is recommended that this filtering be confined to approximately the last quarter of the treatment inasmuch as by that time substantially all of the moisture present has been absorbed by the fabrics being cleaned.

It is of great importance that the absorbefacient employed in the process have the capacity to pass the filters in solution. Otherwise the process would not be adapted for use in the modern, well-equipped dry cleaning plants, in practically all of which filtration during treatment is standard practice. The absorbefacient, therefore, must form in the cleaning solvent a stable, permanent solution which will pass the filters, will not settle out, or change chemically or physically in such wise as to lose its requisite colloidal properties.

The fabrics are next given a rinse in cleaning solvent after which they are dried and subjected to relatively routine handling. The filtration of the cleaning solvent containing the absorbefacient may be continued after the removal of the fabrics until the cleaning solvent is clarified to the desired extent. The cleaning solvent is preferably agitated but not passed through the filter during the addition of moisture for the next batch of fabrics to be treated. As pointed out previously, the amount of moisture added must be predetermined and calculated in relation to the weight and nature of the next batch of fabrics. After the cleaning solvent accumulates too great an amount of oil soluble soil or contamination to be clarified and purified by filtration, it is distilled and a new moisture absorbent solution constituted.

As far as is known, it is necessary to use absorbefacients in all of the cleaning solvents at present available to endow them with the properties requisite for the practice of this invention. These properties desirable for the cleaning solvent include: filterability (in the absence of moisture); power and capacity to repeatedly absorb substan-

tial quantities of moisture in a state of subdivision so fine that the solution is substantially optically clear; chemical inertness towards all varieties of fibres, dyestuffs, sizes and finishes; physical and 5 chemical stability.

The term "absorbefacient" is used throughout this disclosure and the claims to indicate a body which dissolves in a cleaning solvent which does not readily absorb any substantial quantity of 10 moisture and renders it capable of absorbing a substantial quantity of moisture.

The problem of constituting such a cleaning solvent is believed to be, at present, beyond the ordinary skill of colloidal chemists, and surely 15 beyond the skill of the dry cleaning industry. Therefore, for the purpose of assisting the skilled in the art in practicing this invention, a number of formulae for absorbefacients is provided. The claims in the present case are, therefore, limited 20 entirely to the art or method, or process of cleaning fabrics herein disclosed. These formulae of absorbefacients are as follows:

|                                                | Per cent |
|------------------------------------------------|----------|
| (1) Sulfonated castor oil containing 31% water | 30       |
| Oleic acid                                     | 21       |
| Potassium oleate                               | 9        |
| Water                                          | 3        |
| Naphtha                                        | 29.5     |
| Hexa hydro phenol                              | 7.5      |
|                                                | 100.0    |

The ratio of absorbefacient to cleaning solvent can be varied, but a 10% concentration is recommended.

|                                              | Per cent |
|----------------------------------------------|----------|
| (2) Sulfonated castor oil, 15% water content | 50       |
| Oleic acid                                   | 50       |

A 16% by weight concentration in cleaning naphtha gives a clear solution which re-absorbs moisture, but the mix is cloudy in concentrations below and above 16%.

|                                                                                                         | Per cent |
|---------------------------------------------------------------------------------------------------------|----------|
| (3) Sodium salt of sulfonated oleic acid naphthalene condensation product—neutralized Twitchell reagent | 42.8     |
| Sodium oleate                                                                                           | 22.0     |
| Oleic acid                                                                                              | 22.0     |
| Ethylene glycol, mono-butyl-ether                                                                       | 13.2     |

A 10% solution of the above formula in cleaning naphtha produces a cleaning solvent capable of containing 1% moisture. The percentage concentration of this absorbefacient in the cleaning solvent is critical.

|                                        | Per cent |
|----------------------------------------|----------|
| (4) Hydrogenated sulfonated anthracene | 14.5     |
| Naphtha                                | 40.5     |
| Oleic acid                             | 17.5     |
| Water                                  | 15.0     |
| Sodium oleate                          | 12.5     |

An 8% concentration in naphtha is recommended. After being depleted of moisture, the solution reabsorbs it, but considerable agitation is required.

|                                        | Per cent |
|----------------------------------------|----------|
| (5) Sulfonated hydrogenated anthracene | 7.55     |
| Naphtha                                | 21.00    |
| Oleic acid                             | 25.60    |
| Water                                  | 11.75    |
| Potassium oleate                       | 26.25    |
| Mono-butyl-ether of ethylene glycol    | 7.85     |

This formula absorbs moisture very readily and

its concentration in the naphtha solution is not critical. A 10% concentration is recommended.

|                                | Per cent |
|--------------------------------|----------|
| (6) Oleic acid                 | 25       |
| Naphtha                        | 25       |
| Pure mahogany sodium sulfonate | 50       |

This material re-absorbs the moisture readily and can be used in any cleaning solvent suitable for dry cleaning in almost any proportions. A 10 recommended concentration is 6%.

|                     | Per cent |
|---------------------|----------|
| (7) Oleic acid      | 35.3     |
| Naphtha             | 35.3     |
| Cyclohexanol        | 17.6     |
| Potassium hydroxide | 5.3      |
| Water               | 3.5      |
| Triethanolamine     | 3.0      |

A 6% solution is suitable for absorbing the 20 usually desirable amounts of moisture.

|                                  | Per cent |
|----------------------------------|----------|
| (8) Oleic acid                   | 30.0     |
| Naphtha                          | 45.0     |
| Ethylene glycol mono butyl ether | 15.0     |
| Potassium hydroxide              | 5.0      |
| Water                            | 5.0      |

A 6% solution is suitable for absorbing the usually desirable amounts of moisture.

These various formulae exhibit to varying degrees the properties of the ideal absorbefacient to be used in practicing this invention. Certain ones of the absorbefacients tend to cause bleeding of some dyestuffs on certain fabrics but are entirely satisfactory for other classes of articles. 35 The use of some of the absorbefacients would require appreciable expert control of the conditions of the cleaning process to insure best results or would be usable only where this control was available. 40

Of the various formulae provided, No. 6 is the preferred and recommended one because it possesses all of the requisite properties previously discussed, can be used with all of the types of cleaning solvents at present employed for dry 45 cleaning, can be used safely and successfully on a commercial scale without supervision of the cleaning process by skilled chemists, and can be used successfully on all types of fabrics adapted to be cleaned by this general process. 50

Moreover, Formula No. 6 may be used in most dry cleaning plants as at present constituted without any substantial changes of equipment or material changes in handling and routing the fabrics through the plant except as herein 55 specified.

Formulae Nos. 7 and 8 are characterized by very ready absorption of moisture and are suitable for use for fabric cleaning purposes without the exercise of an undue amount of chemical 60 control. These formulae are characterized by the use of partially saponified oleic acid and a material or reagent mutually miscible with oil and water. This reagent may be termed an absorption 65 assistant. Cyclohexanol is the absorption assistant of Formula No. 7 and ethylene glycol mono butyl ether of Formula No. 8. Other mutually miscible materials which may be used as absorption assistants (though with varying degrees of safety on dyed fabrics), comprise butyl 70 acetate, isopropyl alcohol, ethyl alcohol, diacetone alcohol, ethylene glycol mono ethyl ether acetate, and diethylene glycol mono butyl ether. Absorption assistants which tend to be taken up by the fabrics must be periodically replenished. 75

5 In regard to these Formulae Nos. 7 and 8, it must be noted that the presence of free fatty acid is desirable to render a fatty acid soap truly soluble in the cleaning solvent in the presence of moisture, and that the absorption assistants augment the power to take up the required quantities of moisture rapidly and in the proper condition of dispersion.

10 Mahogany sulfonates are the salts of mahogany acids which are formed in the oil layer or A layer in the refining of medicinal white oil and the like by the use of fuming sulfuric acid and/or sulfur trioxide. The United States Patent to Divine, No. 1,493,111, issued May 6, 1924, discloses 15 mahogany sulfonic bodies suitable for the practice of this process.

20 Great care must be used in employing this invention with chlorinated cleaning solvents to avoid the formation of harmful quantities of hydrochloric acid and therefore throughout this 25 description the invention has been disclosed in relation to the equipment of an open, naphtha-process plant, though it must be understood that other types of equipment and plants may be used with appropriate minor modifications well within the skill of the art.

30 I have observed that in the actual practice of the process herein disclosed in commercial dry cleaning plants, silk or rayon fabrics (or in mixture thereof) which have been finished with water sensitive sizes such as the starch or dextrine sizes are very much improved in appearance. In fact, the fabrics frequently look much better than they did when they were absolutely new. 35 The moisture which is absorbed by the fabrics in the process seems to revitalize the size, seems to level it to compensate for size which may have been removed by wear, and altogether restores the uniformity of the finish of the fabric and provides a lustre which is highly attractive and desirable. By this it is meant that not only is water soluble soil removed from the fabrics in the cleaning process but that the physical condition of the finish of the fabrics is actually changed.

40 45 50 55 Claims directed to the general dry cleaning process herein disclosed, including claims directed broadly to humidifying the cleaning solvent, or using an absorbefacient for charging the solvent with moisture in relation to the batch being cleaned, appear in my original co-pending application Serial No. 590,981, now issued into Patent No. 1,911,289, dated May 30, 1933, whereas the claims of this application are all directed to a method of affecting the appearance of fabrics finished with water sensitive sizes.

Having described the invention, I desire to be limited only by the following claims.

I claim:

1. The process of leveling the size of silk and 60 rayon fabrics finished with a water sensitive size,

said process comprising, agitating said fabrics in a dry cleaning solvent of the group consisting of volatile and chlorinated hydrocarbons in which there is dispersed moisture equal in amount to between five and fifteen percent of the weight of the 5 fabrics being treated, and continuing said agitation until the fabrics being treated have absorbed said moisture from the dry cleaning solvent.

2. The process of leveling and brightening the 10 appearance of silk and rayon fabrics finished with a water sensitive size, said process, comprising, agitating said fabrics in a dry cleaning solvent of the group consisting of volatile and chlorinated hydrocarbons in which is dispersed moisture in amount equal to between five and fifteen percent 15 of the weight of the fabrics.

3. A new art of leveling the size and brightening the appearance of silk and rayon fabrics finished with water sensitive sizes, said art comprising, treating said fabrics in an optically clear 20 dispersion of moisture in a cleaning solvent of the group consisting of volatile and chlorinated hydrocarbons, the weight of the moisture dispersed in said solvent plus the weight of the moisture already in the fabrics being equal to 25 between substantially five and fifteen percent of the weight of the fabrics.

4. The process of leveling the size of silk or rayon fabrics finished with water sensitive sizes, comprising, removing substantially all of the 30 moisture from the fabrics, then agitating said fabrics in a dispersion of moisture in a cleaning solvent selected from the group consisting of volatile and chlorinated hydrocarbons, said solvent being substantially optically clear, the dispersed moisture being equal to between substantially 35 five and fifteen percent of the weight of the fabrics being treated.

5. The method of leveling water sensitive sizing of silk and rayon fabrics without removing said 40 sizing from said fabrics, comprising, causing said fabrics to absorb evenly and uniformly from substantially 5 to 15% of moisture based on the weight of said fabrics by treating said fabrics with a very fine dispersion of moisture in an organic dry cleaning solvent of the group consisting of volatile and chlorinated hydrocarbons. 45

6. The method of leveling water sensitive sizing of silk and rayon fabrics without removing said sizing from said fabrics, comprising, causing said 50 fabrics to absorb evenly and uniformly a quota of moisture appropriate to level said sensitive sizing, but not exceeding substantially 15% of moisture based on the weight of said fabrics, by treating said fabrics with a very fine dispersion 55 of moisture in an organic dry-cleaning solvent of the group consisting of volatile and chlorinated hydrocarbons.